

Jan. 26, 1960

G. KOSTYREFF

2,922,758

METHOD OF CONVERTING CRANK CASE OIL TO USABLE OIL

Filed May 8, 1958



INVENTOR  
*George Kostyreff*  
BY  
*Michael S. Stricker*  
ATTORNEY

**1**

2,922,758

**METHOD OF CONVERTING CRANK CASE OIL TO USABLE OIL**

George Kostyreff, New York, N.Y., assignor of one-half to Irving B. Guller, New York, N.Y.

Application May 8, 1958, Serial No. 733,955

13 Claims. (Cl. 208—183)

The present invention relates to a method of converting crank case oil to usable oil, and more particularly to a method of removing impurities from used oil such as crank case oil so as to produce a pure oil which can be used for a variety of different purposes.

Used oil from machinery such as automobile engines and the like, such used oil generally being referred to as crank case oil, constitutes a great waste of our natural resources. Such used oil contains many impurities such as water, dust, lint, metal filings, metal oxides, tars, pitch, etc. which prevent further use of the oil without damage to the engine or the like. Many attempts have been made to develop processes for removing these impurities from the oil in order to obtain an oil which can be reused. In general it may be stated that all of the processes to date involve such high expenses that it is commercially impractical to purify such used oils, and consequently for the most part such used oils constitute a great waste.

It is, therefore, a primary object of the present invention to provide a method of converting used oil, i.e. crank case oil, to a usable oil in a manner which is so inexpensive that it is now commercially practicable to obtain usable oil from such used oil.

It is another object of the present invention to provide a method of converting crank case oil to usable oil whereby the resulting usable oil has properties at least equal to the properties of the original oil before use of the same.

It is still another object of the present invention to provide an inexpensive method of converting crank case oil to usable oil whereby the crank case oil is dehydrated and impurities are removed without resulting in great loss of the good oil of the crank case oil.

Other objects and advantages of the present invention will be apparent from a further reading of the specification and of the appended claims.

With the above objects in view, the present invention mainly comprises a method of converting used oil to usable oil wherein the used oil is dehydrated by evaporation of the water contained therein, the dehydrated oil is treated with sulfuric acid, the sludge is separated from the clear oil, the clear oil is subjected to treatment with adsorbents with heating and steam, and then filtered to result in the production of pure oil that may be reused for all purposes for which the original oil could be used.

The novel features which are considered as characteristic for the invention are set forth in particular in the appended claims. The invention itself, however, particularly with respect to complete details as to the method of proceeding, will be best understood from the following description of specific embodiments. The accompanying drawing which constitutes a flow sheet sets forth further details as to the method of the present invention which will herein be described in still greater detail.

Referring first to the flow sheet it will be seen that a complete method of operation including all stages for the

**2**

obtention of a final product of superior quality, certain of the stages of which can be omitted while still obtaining a usable final product, is set forth.

It will be noted that the flow sheet outlines the various stages of the process of the present invention. In the following each of the stages will be discussed in greater detail:

**DEHYDRATION OF CRANK CASE OIL BY HEATING TO ABOVE BOILING POINT OF WATER BUT BELOW DISTILLATION TEMPERATURE OF OIL FOLLOWED BY SLIGHT COOLING TO PROMOTE SEPARATION, AND REPEATING UNTIL OIL IS DEHYDRATED.**

15 The crank case oil is first dehydrated by evaporation of the water therefrom. This method of drying not only removes water but also removes benzene. Since the presence of benzene or water is undesirable with respect to subsequent treatment with sulfuric acid, drying by means of drying agents such as calcium chloride and aluminum chloride without evaporation would not be as satisfactory as drying by evaporation of the water (which also results in the removal of benzene and other substances which would have a deleterious effect on the subsequent sulfuric acid treatment).

20 As indicated above, the temperature used for the dehydration should be as high as possible, e.g. above the boiling point of water, in order to effect the most rapid dehydration possible, time being most important from the standpoint of economy. However, the temperature should not be so high as to cause distillation or cracking of the oil.

25 While it is desirable to carry out such dehydration under vacuum, and as a matter of fact under the lowest possible pressure, in order to separate as much as possible the dehydration temperature from the distillation temperature, the use of vacuum treatment requires increased apparatus costs and increased energy costs. Accordingly, under the preferred embodiment of the present invention 30 the dehydration is carried out at normal pressure. According to this embodiment the crank case oil is heated to above the boiling point of water but not above 105° C. Most preferably the heating is to a temperature of 104° C.

35 In order to promote separation of the water from the oil without blowing away excessive amounts of the oil the crank case oil is heated up to 105° C., preferably up to 104° C. while stirring and then cooled to about 96—100° C. (preferably 100° C.) without stirring. In this manner some of the water remains at the bottom of the 40 container and can be drawn off through a tap located at the bottom of the container. The heating to 105° C. and cooling to 100° C. is repeated several times until the oil is dehydrated. The end of the dehydration is observable when foam no longer appears upon heating from 100° C. to 105° C. (this heating being carried out while stirring).

45 The number of times of heating to 105° C. and cooling to 100° C. until dehydration depends upon the particular impurities in the oil, e.g. the presence of hygroscopic bodies. Generally repetition of the treatment from two to six times is sufficient, repetition for four times being average for most crank case oils.

**COOLING OF DEHYDRATED OIL**

50 The dehydrated oil is then cooled preferably to a temperature of 10° C. or less and if possible to a temperature as low as 0° C. or less. It is possible to allow the temperature to drop without external cooling means to as low as 40° C. or less before applying external cooling. During the cooling there is some settling of sludge, and 55 this may be removed.

MIXING OF PORTIONS OF DEHYDRATED OIL  
WITH SULFURIC ACID AND SETTLING—SUBSEQUENT PORTIONS BEING ADDED TO ALREADY SETTLED PORTIONS

The cooled, dehydrated oil is then treated with sulfuric acid to remove impurities in the form of a sludge which can be separated from the clear oil by decantation or by withdrawal of the sludge from the bottom of the container. In either case the sludge must be permitted to settle fully and such settling is promoted in accordance with the present invention by a special batch treatment of the dehydrated oil with sulfuric acid.

In accordance with this embodiment of the invention a portion only of the cooled, dehydrated oil, e.g. one fifth thereof, is thoroughly mixed with the sulfuric acid e.g. for about one hour and this portion is then placed in a container to permit settling of the sludge. While the sludge is settling in this portion, a subsequent portion is thoroughly mixed with sulfuric acid e.g. for about one hour. This subsequent portion is then added to the container containing the already settled portion. It has been found that the already settled mixture of sludge and clear oil promotes the settling of the subsequently added mixture of sludge and oil.

Although the present invention is not meant to be limited as to any theory of why or how the already settled oil promotes more rapid settling of the subsequently added mixture of sludge and oil, the following theory is given in the hope that it will help others to better understand the invention. Upon settling of the oil-sludge mixture the densest portion settles to the bottom and the density of the settled layer progressively decreases from bottom to top. The subsequently added mixture of sludge and oil has a greater density than the upper layer of the already settled oil. Consequently, the heavier portions of the subsequently added mixture (charged with concentrated sulfuric acid) very quickly move towards the bottom of the container. Thus, the second portion which has the same volume as the first portion actually settles more rapidly than the first portion. Moreover, the total time of settling of the first and second portions is less than would be the time required for settling of the two portions if originally mixed together with the sulfuric acid.

Further batches of the cooled, dehydrated oil are then mixed with the sulfuric acid and each added separately to the already settled oil, each subsequent batch being added only after the previous batch has already settled. Not only is the settling more rapid by proceeding in this manner, but of at least equal importance, the settling is more complete.

The number of batches may vary within wide limits, the greater the number of batches, the more complete the separation of the sludge from the oil. However, in order to reduce operating time at the start of operation in a plant, the operating time being greater with a larger number of batches at the start of operation because each batch must be thoroughly mixed with the sulfuric acid for the full time, although subsequent treatment time would be reduced, the total number of batches into which the original oil is divided should not be unduly high. For practical purposes division into 3-25 batches is suitable, and most preferably the number of batches should be from 5-8.

The cooled, dehydrated oil is treated with highly concentrated sulfuric acid, i.e. sulfuric acid having a concentration of at least 66° Baumé. The amount of sulfuric acid may vary between 1-10% by volume of the volume of oil treated. Preferably the amount of sulfuric acid varies between 1-2% by volume.

The sulfuric acid used in this treatment should preferably be free of selenium.

SEPARATION OF SLUDGE FROM CLEAR OIL

The sludge is separated from the clear oil by draw-

ing off the sludge at the bottom of the container. If desired the purified oil may be subjected to a second or even a third fractional acid treatment of the type described above, the oil of course being permitted to settle and the sludge being separated between acid treatments. After the first or second acid treatment the oil may be treated with 1-2% of fuming sulfuric acid, e.g. 10% fuming sulfuric acid (10%  $\text{SO}_3 + \text{H}_2\text{SO}_4$ ) for about 10-15 minutes. After settling and the drawing off of the sludge the oil may be treated with 1-2% of fuming sulfuric acid of increasing concentration, e.g. 15-20% fuming sulfuric acid. This method of operation may be used to produce completely decolorized oil.

As stated above, the concentrated sulfuric acid used for the original treatment should be free of selenium. It should also be free of  $\text{H}_2\text{SeO}_3$  and  $\text{MnO}_2$ . If the sulfuric acid is used in small volume it may contain significant amounts of chromic acid (which is likely to oxidize alcohols to acids). If large amounts of sulfuric acid are used only very small amounts of chromic acid should be present.

MIXING OF CLEAR OIL WITH ADSORBENT SUCH AS FULLER'S EARTH AND HEATING

The clear oil separated from the sludge is mixed with an adsorbent such as coarsely purified, non-acid treated fuller's earth. The purpose of the adsorbent is of course to remove impurities and therefore the amount of the adsorbent is not particularly critical. However, in order to facilitate subsequent treatment and separation of the adsorbent-sludge from the liquid the amount of adsorbent is preferably maintained at between 3-6% by weight.

It is in addition particularly advantageous to use non-acid treated fuller's earth as the adsorbent in order to adsorb all of the free sulfuric acid. The non-acid treated fuller's earth when mixed with the acid-treated oil not only removes the free sulfuric acid, but by reason of adsorption of the free sulfuric acid becomes converted into activated fuller's earth. The latter acts upon the remainder of the sludge to remove a portion of the impurities.

Thus, the treatment with non-acid treated fuller's earth is further economical in that it replaces two steps which would otherwise be necessary, namely, neutralization by washing (with all of the disadvantages resulting therefrom), and treatment with activated fuller's earth. In addition to economy the process of the present invention is further advantageous in that after treatment of the oil with non-acid treated fuller's earth the oil does not smell, whereas if the acid treated oil were neutralized by washing and then treated with activated fuller's earth the oil would still have a bad odor.

However, it is possible to use instead of the non-acid treated fuller's earth another adsorbent such as Super Filtrol, bone black, blood charcoal, amorphous carbon, Floridin, frankonite and other hydrosilicates originating by decomposition of hornblendes and augites. It is also possible to use instead of the above adsorbents activated aluminum (produced by melting aluminum and pouring the liquid molten aluminum into cold water), or another metal which is capable of a substratum amorphous effect.

The use of activated aluminum as an adsorbent is advantageous by reason of the fact that the activated aluminum can be easily reconditioned for further use. However, when activated aluminum is used special precautions should be taken to avoid explosions during subsequent treatment. Activated aluminum not only adsorbs ketones, aldehydes and carbon (both colloidal and free) but upon contact with acids it forms hydrogen. Therefore, when activated aluminum is used care should be taken to remove all of the sludge including the activated aluminum from the oil before the oil reaches any distilling drum where it is subjected to high temperature treatment.

The readily available and inexpensive fuller's earth is particularly suitable for reasons of economy. Fuller's

earth having the following composition may be used, for example:

|                                                        | Percent    |
|--------------------------------------------------------|------------|
| SiO <sub>2</sub>                                       | 44 to 72   |
| Al <sub>2</sub> O <sub>3</sub>                         | 5 to 33    |
| Fe <sub>2</sub> O <sub>3</sub>                         | 1.2 to 15  |
| CaO                                                    | 0.3 to 7.4 |
| MgO                                                    | 0.4 to 4.3 |
| K <sub>2</sub> O + Na <sub>2</sub> O                   | 0.4 to 8.3 |
| H <sub>2</sub> O                                       | 4.3 to 25  |
| P <sub>2</sub> O <sub>5</sub> , SO <sub>3</sub> , etc. | Traces     |

The mixture of clear oil and adsorbent is heated under constant stirring to a temperature of 130 to 210° C., and preferably to a temperature of about 180° C.

#### Cooling, Settling and Separating Sludge From Clear Liquid

After the thorough mixing and heating of the oil with the adsorbent the stirring is stopped and the mixture is permitted to cool and settle. The sludge is then separated from the clear oil by careful drawing off of the sludge. The separation of the sludge from the oil may be carried out at any suitable temperature e.g. from 15° C. to 160° C. In order to minimize heat waste, in view of the fact that after this stage the oil is again heated, it is advisable to separate the sludge from the clear oil as soon as possible after settling of this sludge, i.e. while the mixture is still relatively hot.

#### Mixing Clear Oil with Adsorbent, and Heating with Steam

The now partially purified oil is again mixed with an adsorbent such as Super Filtral, preferably in an amount of 1% to 3% by weight, and most preferably about 2% by weight. At least 2% by weight of this adsorbent should be used if the previous treatment was carried out with activated aluminum.

Instead of Super Filtral it is suitable to use Tonsil, kieselguhr, and various other kinds of German clay, or the like.

The mixture of oil and adsorbent is heated under vacuum with steam injection. The higher the pressure (i.e. the lower degree of vacuum) the more steam should be used. The pressure during this treatment should be preferably 100 mm. Hg or less, and most preferably 50 mm. Hg or less. The temperature during this treatment may vary between, preferably 275-337.5° C. The amount of steam measured as condensed water is preferably 2 to 20 volumes per each volume of oil, depending upon the temperature and pressure.

As the oil-adsorbent mixture is heated to higher temperatures the pressure must be lowered. At a temperature of up to 220° C. the pressure may be up to 100 mm. Hg. As the temperature is increased up to 275° C. the pressure should be maintained at up to 50 mm. Hg. As the temperature increases the injection of steam should also be increased and higher amounts of steam should be used at higher pressures. At a temperature of 200-275° C. the amount of steam as condensed water is preferably 10 to 20 volumes per volume of oil, at 50-100 mm. Hg.

At lower pressures of less than 50 mm. Hg e.g. as low as 10 mm. Hg or less, and at temperatures of up to 337.5° C. the amount of injected steam may be 2 to 4 volumes per volume of extracted oil.

At reduced pressures of about 10 mm. Hg it is possible to use helium to substitute for some of the steam.

In order to lower expenses the degree of vacuum is not made excessively high, e.g. the pressure may be maintained at about 50 mm. Hg. When carrying out the process at this pressure the steam injection should be started at about 220° C., increased at about 275° C. and still further and greatly increased from 310 to 337.5° C.

During this stage of the proceeding the adsorbent not only has an action in adsorbing impurities, but also in

providing for a correct dispersion of the introduced steam. The high temperature and vacuum treatment not only has the effect of removing diluent, but also removes a noticeable amount of impurities by distillation. The extracted oil, particularly that fraction obtained at a temperature up to 275° C. may be used as a fuel for tractors and the like.

#### Cooling, Settling and Separating Sludge From Clear Liquid

The heated mixture of oil and adsorbent is then cooled. The steam injection is continued until the mixture starts to be cooled to below 220° C. Preferably the steam injection is continued until the temperature reaches 160° C.

At the same time the mixture is permitted to settle and as soon as the settling is sufficiently complete the sludge is drawn off. For reasons of economy, to effect a saving in both time and heat, it is desirable to draw off the sludge at a temperature as high as possible, e.g. up to 150° C. Of course, the separation of the sludge from the clear oil can be carried out at lower temperatures, e.g. as low as 20° C.

#### Mixing Clear Oil with Adsorbent and Heating (Without Steam)

The clear oil is then mixed with an adsorbent. It is preferred at this stage of the proceeding to use an adsorbent of high decolorizing properties such as Retrol which is an acid-activated montmorillonite adsorbent. Among other suitable adsorbents may be mentioned Tonsil, Norite or the like. The amount of adsorbent such as Retrol is preferably 1-5%, the lower amount being preferred for reasons of economy.

The mixture of oil and adsorbent is heated, with thorough stirring, without steam, to a temperature of 130-230° C.

#### Cooling, Settling and Separating Sludge From Clear Liquid Oil

The mixture is then cooled and allowed to settle. After settling the sludge is drawn off. The sludge may be drawn off at a temperature as high as 180° C. or as low as 5° C. The separation of the sludge from the clear oil may be carried out by drawing off the sludge at the bottom of the container or by decantation.

#### Filtrating Oil and Deodorizing, If Necessary

The oil may then be filtered, e.g. using a filter press. The filtered oil may also be deodorized, for example by reheating up to 130° C. and preferably up to 105° C., followed by steaming until no odor is apparent. This deodorizing treatment does not affect the quality of the oil.

By proceeding in the above described manner, ordinary crankcase oil containing such impurities as heavy organic acids, anhydrides and esters thereof, oxy-acids, estolides, wax-alcohols, aldehydes, ketones, fats which were added for consistency, kerosene, gasoline, mazout, lanoline and sulfur which are added to the oils by large firms, detergents, benzene absorbed in cars which do not use the full speed run, water, dust, cotton particles, metal filing, metal oxides, metals in colloidal state, tars, pitches, carbon (both colloidal and in suspension) etc., are purified and reconditioned to produce oils which have the quality of the best oils presently on the market. As a matter of fact some of the reconditioned oils produced in accordance with the present invention are actually superior to the usual commercial oils. The major portion of the reconditioned oils produced in accordance with the present invention is composed of saturated normal chain hydrocarbons which actually prevent engine deterioration in a superior manner to new oils. Engine test runs have shown that reconditioned oils produced according

to the present invention do not heat motors to the same

extent as the new oils, which indicates that the reconditioned oils of the present invention no longer contain constituents which can be converted to acid constituents. Furthermore, the lubricating properties of the reconditioned oils of the present invention are superior to new oils. It is believed that this is due to the fact that the new oils are actually to some extent purified as they are used in an engine. Thus, when the oils are reconditioned according to the present invention they have already been purified to some extent by use in an engine, and accordingly the final reconditioned oil has superior properties.

The following example is given to further illustrate the present invention. The scope of the invention is not, however, meant to be limited to the specific details 15 of the example.

*Example*

20 liters of ordinary crank case oil are heated in an open vessel under constant stirring to a temperature of 20 104° C. When the temperature reaches 104° C. the heating is stopped and the oil permitted to cool to 100° C. While still stirring the heating is again started and the oil is heated to 104° C. The heating is again stopped, and the oil cooled to 100° C. This cycle is repeated three 25 additional times, the total time of the treatment requiring one hour.

The oil is then cooled by means of an external cooling means such as ice to a temperature of about 5° C.

4 liters of the cooled oil are mixed for one half hour, 30 utilizing a stirrer revolving at 800 revolutions per minute, with 100 grams of 66° Baumé sulfuric acid. The stirring is continued for one half hour. The acid treated oil is then drawn off into a settling vessel.

An additional 4 liters of cooled oil are mixed for one half hour in the same manner as above with 100 grams of 66° Baumé sulfuric acid for one half hour. By this time the first 4 liters of oil has settled. The second 4 liters of oil are added to the first 4 liters of oil in the settling vessel.

The operation is continued until the entire 20 liters has been acid-treated and drawn off into the settling vessel, the total time being two and one half hours. The acid-treated oil is then permitted to settle for an additional six hours and the settled oil is decanted into another vessel.

60 600 grams of coarsely purified, non-acid treated fuller's earth is added and the mixture is heated under constant stirring to a temperature of 180° C. The heating and the stirring are both stopped and the mixture is permitted to settle and cool. By the time the temperature reaches 140° C. the mixture is settled sufficiently to permit decanting of the supernatent clear oil.

The clear oil is mixed with 200 grams of Super Filtral and in a steam injection vacuum apparatus heated at a pressure of 50 mm. Hg to a temperature of 310° C., the amount of steam introduced during this heating amounting to 40 liters of water. The heating is stopped and the mixture permitted to cool to a temperature of 140° C., the steam injection continuing until the temperature has reached 150° C. The sludge is drawn off at the bottom and the oil is then tapped off.

65 The oil is mixed with 400 grams of Retrol and heated to 200° C. The heating is discontinued. When the mixture cools to 150° C. it has settled sufficiently to permit decanting of the supernatent clear oil. The clear oil is steamed, heated to 110° C. and passed through a filter press.

70 16 liters of clear oil having properties equivalent to fresh oil are obtained. The oil may be used in cars as a motor oil of superior quality.

Without further analysis, the foregoing will so fully reveal the gist of the present invention that others can by applying current knowledge readily adapt it for various applications without omitting features that, from the 75

standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. A method of producing usable oil from used oil, comprising the steps of heating used oil at a temperature above the boiling point of water and below the distillation temperature of the oil so as to dehydrate said oil; cooling said dehydrated oil; mixing a first portion of said dehydrated, cooled oil with sulfuric acid so as to form of said first portion, a mixture of oil and a sludge containing impurities; permitting the thus formed mixture to settle; successively mixing further portions of said dehydrated, cooled oil with sulfuric acid and successively adding the thus formed further portions of oil and sludge to said first portion until the whole of said oil has been mixed with sulfuric acid and added to said first portion, the already settled portions promoting the settling of subsequently added portion; permitting the thus formed mixture to settle; separating said sludge from said oil; treating the thus obtained oil by mixing the same with an adsorbent and heating so as to cause adsorption of impurities by said adsorbent, thereby forming a mixture of clear oil and sludge; and separating said sludge from said clear oil, thereby obtaining a clear oil of high quality.

2. A method of producing usable oil from used oil, comprising the steps of heating used oil at a temperature above the boiling point of water and below the distillation temperature of the oil so as to dehydrate said oil; cooling said dehydrated oil; mixing a first portion consisting of one-third to one twenty-fifth of the whole of said dehydrated, cooled oil with sulfuric acid so as to form of said first portion a mixture of oil and a sludge containing impurities; permitting the thus formed mixture to settle; successively mixing further portions of said dehydrated, cooled oil with sulfuric acid and successively adding the thus formed further portions of oil and sludge to said first portion until the whole of said oil has been mixed with sulfuric acid and added to said first portion, the already settled portions promoting the settling of subsequently added portion; permitting the thus formed mixture to settle; separating said sludge from said oil; mixing the thus obtained oil with an adsorbent and heating the mixture so as to cause adsorption of impurities by said adsorbent and form a mixture of oil and sludge; permitting said mixture to settle; separating the thus settled sludge from said oil; mixing the thus obtained oil with an adsorbent so as to form a mixture thereof; heating said mixture in the presence of steam so as to cause adsorption of impurities by said adsorbent, thereby forming a mixture of clear oil and sludge; and separating said sludge from said clear oil, thereby obtaining a clear oil of high quality.

3. A method of producing usable oil from used oil, comprising the steps of heating used oil at atmospheric pressure at a temperature between 100-105° C. while agitating; cooling the thus heated oil to a temperature of 96-100° C.; repeating said heating to 100-105° C. and cooling to 96-100° C. until said oil is dehydrated; cooling said dehydrated oil; treating said dehydrated, cooled oil with sulfuric acid, thereby forming a mixture of oil and a sludge containing impurities; separating said sludge from said oil; treating the thus obtained oil by mixing the same with an adsorbent and heating so as to cause adsorption of impurities by said adsorbent, thereby forming a mixture of clear oil and sludge; and separating said sludge from said clear oil, thereby obtaining a clear oil of high quality.

4. A method of producing usable oil from used oil, comprising the steps of heating used oil at atmospheric pressure at a temperature between 100-105° C. while agitating; cooling the thus heated oil to a temperature of 96-100° C.; repeating said heating to 100-105° C.



acid and added to said first portion; permitting the thus formed mixture to settle; separating said sludge from said oil; mixing the thus obtained oil with an adsorbent so as to form a mixture thereof; heating said mixture in the presence of steam so as to cause adsorption of impurities by said adsorbent, thereby forming a mixture of oil and sludge; permitting said mixture to settle; separating the thus settled sludge from the oil; mixing the thus obtained oil with an adsorbent and heating the thus formed mixture, thereby forming a mixture of clear oil and sludge; separating said sludge from said clear oil, thereby obtaining a clear oil of high quality; and subjecting the thus obtained clear oil to a deodorizing treatment.

11. A method of producing usable oil from used oil, comprising the steps of heating used oil at atmospheric pressure at a temperature between 100-105° C. while agitating; cooling the thus heated oil to a temperature of 96-100° C.; repeating said heating to 100-105° C. and cooling to 96-100° C. until said oil is dehydrated; cooling said dehydrated oil to a maximum temperature of 10° C. mixing a first portion of said dehydrated, cooled oil with sulfuric acid so as to form of said first portion a mixture of oil and sludge containing impurities; permitting the thus formed mixture to settle; successively mixing further portions of said dehydrated, cooled oil with sulfuric acid and successively adding the thus formed further portions of oil and sludge to said first portion until the whole of said oil has been mixed with sulfuric acid and added to said first portion, the already settled portions promoting the settling of subsequently added portions; permitting the thus formed mixture to settle; separating said sludge from said oil; mixing the thus obtained oil with an adsorbent and heating the mixture to a temperature of 130-210° C. so as to cause adsorption of impurities by said adsorbent, thereby forming a mixture of clear oil and sludge; and separating said sludge from said clear oil, thereby obtaining a clear oil of high quality.

12. A method of producing usable oil from used oil, comprising the steps of heating used oil at atmospheric pressure at a temperature between 100-105° C. while agitating; cooling the thus heated oil to a temperature of 96-100° C.; repeating said heating to 100-105° C. and cooling to 96-100° C. until said oil is dehydrated; cooling said dehydrated oil to a maximum temperature of 10° C. mixing a first portion of said dehydrated, cooled oil with sulfuric acid so as to form of said first portion a mixture of oil and sludge containing impurities; permitting the thus formed mixture to settle; successively mixing further portions of said dehydrated, cooled oil with sulfuric acid and successively adding the thus formed further portions of oil and sludge to said first portion until the whole of said oil has been mixed with sulfuric acid and added to said first portion, the already settled portions promoting the settling of subsequently added portions; permitting the thus formed mixture to settle; separating said sludge from said oil; mixing the thus obtained oil with an adsorbent and heating the mixture to a temperature of 130-230° C., thereby forming a mixture of clear oil and sludge; and separating said sludge from said clear oil, thereby obtaining a clear oil of high quality.

to a temperature of 130-210° C. so as to cause adsorption of impurities by said adsorbent, thereby forming a mixture of clear oil and sludge; separating said sludge from said clear oil; mixing the thus separated clear oil with an adsorbent so as to form a mixture thereof; heating said mixture in the presence of steam at a maximum pressure of 100 mm. Hg to a temperature of 275-337.5° C. so as to cause adsorption of impurities by said adsorbent, thereby forming a mixture of oil and sludge; permitting said mixture to settle; separating the thus settled sludge from the oil; mixing the thus obtained oil with an adsorbent and heating the thus formed mixture, thereby forming a mixture of clear oil and sludge; and separating said sludge from said clear oil, thereby obtaining a clear oil of high quality.

13. A method of producing usable oil from used oil, comprising the steps of heating used oil at atmospheric pressure at a temperature between 100-105° C. while agitating; cooling the thus heated oil to a temperature of 96-100° C.; repeating said heating to 100-105° C. and cooling to 96-100° C. until said oil is dehydrated; cooling said dehydrated oil to a maximum temperature of 10° C. mixing a first portion of said dehydrated, cooled oil with sulfuric acid so as to form of said first portion a mixture of oil and sludge containing impurities; permitting the thus formed mixture to settle; successively mixing further portions of said dehydrated, cooled oil with sulfuric acid and successively adding the thus formed further portions of oil and sludge to said first portion until the whole of said oil has been mixed with sulfuric acid and added to said first portion, the already settled portions promoting the settling of subsequently added portions; permitting the thus formed mixture to settle; separating said sludge from said oil; mixing the thus obtained oil with an adsorbent and heating the mixture to a temperature of 130-210° C. so as to cause adsorption of impurities by said adsorbent, thereby forming a mixture of clear oil and sludge; separating said sludge from said clear oil; mixing the thus separated clear oil with an adsorbent so as to form a mixture thereof; heating said mixture in the presence of steam at a maximum pressure of 100 mm. Hg to a temperature of 275-337.5° C. so as to cause adsorption of impurities by said adsorbent, thereby forming a mixture of oil and sludge; permitting said mixture to settle; separating the thus settled sludge from the oil; mixing the thus obtained oil with an adsorbent and heating the thus formed mixture to a temperature of 130-230° C., thereby forming a mixture of clear oil and sludge; and separating said sludge from said clear oil, thereby obtaining a clear oil of high quality.

#### References Cited in the file of this patent

#### UNITED STATES PATENTS

|           |               |               |
|-----------|---------------|---------------|
| 1,564,501 | Weir          | Dec. 8, 1925  |
| 1,707,671 | Aycock et al. | Apr. 2, 1929  |
| 2,563,369 | Reiley et al. | Aug. 7, 1951  |
| 2,585,874 | Stratford     | Feb. 12, 1952 |